

## UNITED STATES PATENT OFFICE.

JOHN STROTHER MILLER, JR., OF RAHWAY, NEW JERSEY, ASSIGNOR TO THE BARBER ASPHALT COMPANY, OF PHILADELPHIA, PENNSYLVANIA, A CORPORATION OF WEST VIRGINIA.

## BASE TABLET FOR SOUND RECORDS.

No Drawing.

Application filed December 13, 1921. Serial No. 522,128.

*To all whom it may concern:*

Be it known that I, JOHN STROTHER MILLER, Jr., a citizen of the United States, and a resident of Rahway, in the county of 5 Union and State of New Jersey, have invented certain new and useful Improvements in Base Tablets for Sound Records, whereof the following is a specification.

Sound producing records for talking machines are ordinarily made of comparatively expensive material, usually a combination of shellac with vegetable fibre. The suitability of this material is due to certain inherent properties permitting its use as a thermoplastic although it is sufficiently hard to withstand the abrasive action of a reproducing needle.

Owing to the expense of this material, efforts have been made to find a suitable material from which may be produced base-tablets of suitable shape and thickness upon the surfaces of which may be placed a coating or facing of the same more expensive material commonly used for the production 25 of the entire sound record. Under these circumstances, the sound record is impressed upon the facing while the base-tablet is merely a vehicle for carrying the more expensive facing with the sound record impressed thereupon. In order, however, to successfully produce such a base-tablet it is necessary to obtain material having a combination of qualities difficult to secure.

I have discovered a material which possesses the combination of strength, toughness, durability, resonance, melting point, coefficient of expansion, and ability to coalesce with or adhere to the facing material which is required for successful use in manufacturing these base-tablets.

My invention consists of a bituminous material having a high melting point intimately and evenly combined with a fibrous material.

According to my invention, I produce a compressed bituminous tablet of suitable shape for receiving the required surfacing, composed of a high melting point bituminous binder combined with a fibrous material 50 such as asbestos fibre, cotton flock or the like thoroughly disintegrated and mixed by grinding with the binder. This material is compressed as usual into a rigid tablet of substantially the same size as the desired finished disk, but slightly thinner, thus per-

mitting the overlay of the facing of fibrated shellac or other mixture suitable for record stock.

For the fibrous material which enters into my improved base-tablet, I have found that it is necessary to employ a fibrous stock which is fairly free from non-fibrous particles. Asbestos fibre is very satisfactory. It is not affected by the high temperature of the melting bitumen. Preferably long-fibred asbestos stock should be chosen and disintegrated to the desired length rather than one of short fibre, produced directly from asbestos rock, which I have found usually contains an objectionable proportion of 70 ground rock.

For the bituminous binder which is to be mixed with this fibrous material, I employ a hard bitumen, having a high melting point. It may be made of certain grades of gilsonite, or else of certain other grades of gilsonite combined with sufficient softening material to produce a material possessing a melting point within the limits of my invention. For example, I may combine 75% of gilsonite with 25% of a petroleum oil asphalt having a melting point of 165° to 190° F. There is thereby produced a bituminous binder having a melting point of not less than 250° F., and preferably between 275° F., and 350° F. I have found that if the binder has a melting point substantially less than 250° F., the resulting base-tablet will not stand up under the temperatures encountered in the subsequent manufacture of the completed record disk. On the other hand, if the binder has a melting point of more than 350° F., the molding of the tablet becomes difficult or impossible owing to temperature and pressure requirements, but between the limits which I have named, the melting point may vary, dependent upon the temperatures available for molding.

The method of compounding my material is as follows:

From 20% to 45% of asbestos fibre, such as I have described, disintegrated before or during the grinding of the mixture, is mixed with 55% to 80% of a bituminous 105 binder made of a composition such as I have described, and lying between the limits of melting point which I have named. These two materials are ground together within a suitable mill either ball or tube 110

mill, until the mixture will all pass a thirty mesh sieve. This powdered mixture is then fused together on a hot mixing mill consisting of horizontal twin rolls steam-heated, one of which rotates more rapidly than the other. When taken from this mixing roll, my material by reason of the qualities of its component parts and the proportions in which they are mixed, is a suitable material to be run through a blanking roll for the manufacture of base-tablets in a manner known in the art. The blanks thus produced are heated on a steam table to a temperature of from 280° to 300° F., and placed in a mold of usual design and compressed. Instead of using a die stamper in the mold, a plain steel surface is used, thus giving a perfectly plain surface to the tablet. As an alternative method of procedure, the finely ground materials may under certain circumstances be fed directly to the heated molds and compressed into the base-tablets.

Base-tablets, such as I have now described, are ready for use in the record-making industry, by subjecting them to the known means for applying record stock to either or both faces, and impressing the record thereon.

Having thus described my invention, I claim:

1. A base tablet for sound records composed of an intimate and even admixture of fibrous material with a bituminous binder having a melting point of not less than 250° F., tough and strong, and adherent to an overlay of thermoplastic record material.

2. A base tablet for sound records com-

posed of an intimate and even admixture of asbestos with a bituminous binder having a melting point of not less than 250° F., tough and strong, and adherent to an overlay of thermoplastic fibrated shellac.

3. A base tablet for sound records composed of an intimate and even admixture of fibrous material with a bituminous binder having a melting point lying between 275° and 350° F.

4. A structural material consisting of from 20% of asbestos fibre evenly mixed with 55% to 80% of a binder consisting of hard bitumen having a melting point lying between 275° and 350° F.

5. A base tablet for sound reproducing records composed of an intimate and even mixture of inorganic fibrous material with a bituminous binder, compressed to ensure rigidity, and adherent to an overlay of thermoplastic record material.

6. A base tablet for sound reproducing records, composed of an intimate mixture of fibrous material and a bituminous binder composed of gilsonite and high melting point petroleum oil asphalt in proportions to produce a mixture having a melting point of not less than 250° F., tough and strong, and adherent to an overlay of thermoplastic record material.

In testimony whereof, I have hereunto signed my name at Maurer, N. J., this 70 second day of December, 1921.

JOHN STROTHER MILLER, JR.

Witnesses:

MICHAEL P. ENNIS,  
WILLIAM FRANCIS KERWIN.